

March 19, 1940.

O. MATTIAT

2,194,183

PIEZOELECTRIC CRYSTAL

Filed June 26, 1937

*Fig. 1*



*Fig. 2*



INVENTOR  
OSKAR MATTIAT

BY *H.S. Grover*  
ATTORNEY

## UNITED STATES PATENT OFFICE

2,194,183

## PIEZOELECTRIC CRYSTAL

Oskar Mattiat, Berlin, Germany, assignor to  
 Allgemeine Elektricitäts Gesellschaft, Berlin,  
 Germany, a corporation of Germany

Application June 26, 1937, Serial No. 150,527  
 In Germany June 29, 1936

## 1 Claim. (Cl. 171—327)

This invention is particularly adapted to monitor circuits of radio frequency transmitters and also is used in connection with cable filters, whereas in the past quartz crystals have been 5 customarily used for such circuits. The use of quartz crystals appeared necessary for the reason that for a long time it has been the only readily workable crystal possessing a sufficiently high piezo electric constant.

10 Now, it has been known in the prior art to cut crystals out of Rochelle salt mother crystals and to use the same in microphones; but it seems also advantageous to use Rochelle salt crystals and other piezo electric crystals such 15 as urotropin as oscillatory crystals, since these crystals are artificially "cultivable", as it were, so that all such difficulties may be obviated as have been encountered in the production of crystals of sufficient purity.

20 According to this invention, rodlets are cut out of the mother crystal of piezo electric salts to be used as oscillatory crystals in such a way that their longitudinal directional will coincide with the direction of least elasticity expressed by 25 modulus of elasticity in tension, or Young's modulus.

The invention shall be explained by reference to the drawing in connection with a Rochelle salt crystal, in which:

30 Fig. 1 illustrates a Rochelle salt crystal with the conventional crystallographic axis designations *a*, *b*, *c*; and

Fig. 2 is a plan view of a plate cut from the crystal.

35 Referring now in detail to the drawing:

In the case of Rochelle salt, the least modulus of elasticity occurs in the plane of the *a*-axis and *c*-axis at an angle of 45 degrees to both axes. Hence, according to the invention a plate 40 *P* must be cut out at right angles to the *b*-axis. The same is again illustrated in Fig. 2. The broken-line curve *E* indicates the size of the modulus of elasticity in terms of polar coordinates. It can be seen therefrom that the lowest elasticity 45 modulus, as stated above, occurs at an angle of 45 degrees. *S* is intended to show in what way a crystal rod according to the invention should be cut out of the plate *P*.

50 Rodlets according to the invention are especially suited as oscillatory crystals. The rod cut out of a Rochelle salt mother crystal according to the instructions hereinbefore disclosed must be of a length of one cm. to be suited for a wave- 55 length of 2100 meters, whereas a quartz crystal

for the same wave-length must be two cm. long. In other words, twice as long. If it were desired to cut a crystal out of a Rochelle salt mother crystal, say, in the direction of the *c*-axis, crystal sizes would be required which are the same as those of the quartz for the same wave-length. Owing to the reduced size, one obtains crystals which, even in the presence of an inherently lower mechanical strength, will exhibit adequate 5 stability in oscillatory state and will thus not break or crack. Tests and research of which the present invention has been the outcome have demonstrated that a crystal of Rochelle salt which had been cut in accordance with the instructions here disclosed is capable of withstanding a load of 15 volts, which is far above the usual stress and load which lies around 1 volt and below.

Another practical merit residing in crystals cut in accordance with this invention is that oscillations due to thrust which would occur in a plate cut, say, in the way of plate *P*, Fig. 2, will thus be avoided so that pure elongation oscillations are obtained. The consequence is an increased purity of the oscillations. The excitation of the crystals, similarly as in quartz, is produced by the aid of two electrodes placed upon the rod, these electrodes being positioned, as will be noted, parallel to the plane through the drawing, Fig. 2. However, while in the quartz crystals vibrations occur in the sense of the electric force, both the undesirable thrust motions of plate *P* as well as the desirable elongational vibrations of the rod *S* occur at right angles to the electrical force.

30 35 40 45 50 55 Crystal rods cut according to the invention are but little dependent upon temperature effect so far as their elasticity modulus and thus their natural frequency is concerned. Under certain circumstances, however, the crystals may be safeguarded from temperature and humidity influences by embedding them in coats of non-hygroscopic substances which are of a nature not to affect the oscillatory properties of the crystal. What has been found serviceable for this purpose are copals.

In order to preclude the chance of producing harmonics and coupling oscillations, the width of the crystal must bear a certain relationship to the length thereof. It has been discovered that suitable oscillatory crystals are obtained if the breadth of the rods is less than one-third their length.

What is claimed is:

A crystal rod cut from piezo electric salts

especially Rochelle salt adapted to be used for oscillatory crystal work, with this characteristic feature that it is cut out of the mother crystal at right angles to the crystallographic *b*-axis at 5 an angle of forty-five degrees to the crystallographic *a*-axis and *c*-axis so that its longitudinal

direction coincides with the direction of the lowest Young's modulus of elasticity and that the width of said crystal rod is less than one-third its length.

OSKAR MATTIAT. 5